# EUROPEAN PATENT APPLICATION

(11) **EP 0 497 042 A2**
(43) Date of publication of application: **05.08.1992**
(21) Application number: 91310544.1
(22) Date of filing: 14.11.1991
(51) Int. Cl.: C23C 18/16, C23C 18/40

(54) **Process and programmable computer controlled system for electroless copper plating**

(30) Priority: 31.01.1991 US 648657
(71) Applicant: MACDERMID INCORPORATED, Waterbury, Connecticut 06702 (US)
(72) Inventor: Martin, Theodore A., Jr., Wolcott, Connecticut 06716 (US)
(74) Representative: Pendlebury, Anthony

(57) **Abstract**

A process for maintaining the level of cyanide ion stabilizer in an electroless copper plating bath held at a constant predetermined temperature by making additions of predetermined amounts of cyanide ion feedstock at predetermined time intervals. The properties of the copper layer deposited on a substrate by means of the system are significantly improved in uniformity and structural strength. In addition, the plating rate and stability of the bath are far more uniform. A programmable computer system for controlling the process of the invention is also described.

## Description

This invention relates to electroless copper plating baths and improved copper plated substrates, and is more particularly concerned with a process and a programmable computer controlled system for electroless copper plating and with substrates coated with copper using said system.

Electroless copper plating of substrates such as printed circuit boards and the like is a well known process. Electroless copper plating baths contain a source of cupric ions, generally copper sulfate, together with a reducing agent such as formaldehyde, a complexing agent for the cupric ion of which ethylenediamine tetra acetic acid (EDTA) is typical, sodium hydroxide to control pH, and various additives such as surfactants and stabilizing agents. A stabilizing agent which is commonly used is a source of cyanide ions such as sodium cyanide.

Underkofler et al U.S. Patent 3,844,799 teach that, by maintaining the cyanide ion concentration of an electroless copper plating bath between 0.0002 and 0.0004 molar, and at the same time maintaining the temperature of the bath between 70°C. and 80°C., it is possible to improve the properties of the deposited copper layer. The range of concentration of cyanide ion called for by this teaching is sufficiently broad to permit variations of up to 100 percent.

No details are given in the above patent as to how the concentration of cyanide ions was monitored in order to make additions to keep the concentration in the required range. A common method of analysis for cyanide ions employs a cyanide ion specific electrode and measures the rate at which silver metal is removed from a membrane in contact with the solution containing the cyanide ion. The accuracy of this method is affected by the presence of ions which may be present in the bath as additives or impurities. For example, the presence of ions such as sulfide, halide, thiocyanate or any ion which forms an insoluble complex with silver, can cause significant interference with an accurate determination of the actual cyanide concentration, particularly where the latter is at a level as low as 0.0002 molar. Other methods of analysis include ion chromatography, polarography, colorimetric, kjeldahl, and amperometric titration. In general these methods lack the required accuracy and/or are slow, i.e. require significant time to carry out thereby causing significant delay in correcting a deficiency of cyanide ion in the bath.

This invention is based on the finding that if the pH, cupric ion and reducing agent concentrations are maintained at constant levels in accordance with normal practice in the art, the rate at which the cyanide ion is consumed is directly related to the temperature at which the bath is maintained. The rate of consumption may be different in baths having different compositions, but, in the case of any given bath wherein the above named parameters are maintained constant, the rate of cyanide ion consumption at a given temperature is directly related to said temperature and is reproducible, i.e. the rate at a given temperature shows substantially the same pattern in all baths which have the same chemical composition.

Accordingly, on the basis of the foregoing findings, for a given bath at a given temperature it is possible to predict how much cyanide ion must be added to the bath at any given elapsed time in order to restore the cyanide ion concentration in the bath to the initial desired level. Therefore, once the relationship of rate of cyanide ion consumption at a chosen bath temperature has been determined, it becomes unnecessary to do routine cyanide analysis of that bath, or any other bath of the same chemical composition, during the operating life of the bath in order to determine how much cyanide ion must be added at any given time to maintain a desired cyanide ion concentration.

Based on the above findings, it has become possible in accordance with the invention to develop a system in which the cyanide ion concentration in an electroless copper plating bath can be maintained substantially constant over a prolonged working period without recourse to repeated analysis for cyanide ion in the bath. In consequence, significant variation in cyanide ion content, which has been a feature of prior systems due to the time required for analysis of aliquots and resulting delay in correcting the cyanide ion concentration after a deficiency is determined, has been eliminated. Further, as will be described in detail below, the above findings have made possible the development of an automated system to maintain the desired level of cyanide ion concentration in an electroless copper plating bath.

It has also been found that the copper layer deposited on a substrate in an electroless plating bath operated in accordance with the invention exhibits markedly improved physical properties compared to a copper layer deposited using the same bath but operated without the benefit of the present invention. Likewise, the stability and plating rate of the bath are far more uniform leading to potentially longer bath life and a more consistent product.

The invention, in its broadest aspect, comprises a process for the electroless deposition of copper onto a substrate surface from an electroless copper depositing bath comprising cupric ions, a reducing agent, a complexing agent and a stabilizing agent comprising cyanide ions, which process comprises the steps of:
(a) establishing, for fixed values of cupric ion concentration, reducing agent concentration, temperature and pH of the bath, a characteristic relationship between cyanide ion consumption in the bath and elapsed time of operation of the bath;
(b) substantially uniformly maintaining the bath at the fixed value of temperature;
(c) substantially uniformly maintaining the concentration of cupric ion, the concentration of reducing agent and the pH of the bath at the fixed values thereof; and
(d) adding to the bath over the course of copper deposition therefrom an amount of cyanide ion sufficient to substantially replace the cyanide ion consumed in the bath based on the characteristic relationship established in (a) above, the additions being carried out at time intervals sufficient to substantially uniformly maintain the cyanide ion concentration in the bath at the predetermined level over the course of copper deposition from the bath.

The invention, in a particular aspect, comprises a computer controlled system for carrying out the process of the invention, said system comprising in combination:
an electroless copper plating bath comprising cupric ions, a reducing agent, a complexing agent and a stabilizing agent comprising cyanide ions, said bath also comprising heat control means for adjusting the temperature thereof;
storage means containing cyanide ion feedstock and pump means associated with said storage means for delivering cyanide ions via a feed line to said plating bath;
programmable computer means for monitoring the temperature of said plating bath at a predetermined level and for controlling the addition of predetermined or calculated amounts of cyanide ions at predetermined intervals, said computer means including:
(a) means for producing base reference signals characteristic of a predetermined bath temperature;
(b) sensing means for producing signals characteristic of the temperature of said bath, comparator means producing signals responsive to a difference between said signals so produced and said base reference signals, and means sensitive to said comparator response to cause said heat control means in said bath to make corrective adjustment to the temperature of said bath; and
(c) means for producing at predetermined time intervals signals characteristic of predetermined or calculated amounts of cyanide feedstock to be added to said bath at said predetermined time intervals and means sensitive to said signals to activate said pump means to deliver each of said predetermined or calculated amounts at each of said intervals.

The invention also comprises a method of electroless deposition of copper on a substrate using the above recited process and system and the improved stability and rate uniformity of the bath and properties of the copper layer so deposited.

FIGURE 1 shows a plot of loss of cyanide ion versus temperature of a typical electroless copper plating bath.

FIGURE 2 shows a schematic rendering of a typical computerized control system in accordance with the invention.

FIGURE 3 shows in schematic form a breakdown of the components of the computer means shown in FIGURE 2.

The cyanide ion CN- has an exceptional ability to complex and sequester monovalent copper, so much so that it can even strip a chelating agent such as EDTA from a monovalent copper-EDTA complex. The resultant cuprous cyanide (CuCN) has such stability that it behaves as an inert substance in the plating bath. The cyanide ion reacts with monovalent copper so fast that it will often prevent other destabilizing reactions from occurring in an electroless copper plating bath. However, the cyanide ion will also react with divalent copper in any one of a number of ways which result in consumption of cyanide ion but do not contribute to stabilizing of the plating bath. The following are typical of these undesirable reactions with divalent copper, the cyanide being used in the form of potassium cyanide for purposes of illustration.

CuCN + 2 KCN⇄ Cu(CN)₃⁼ + 2K⁺

Cu(CN)₃⁼ + KCN⇄ Cu(CN)₄⁼ + K⁺

Cu⁺⁺ + 2 KCN→Cu(CN)₂ + 2 K⁺

2 Cu(CN)₂→ 2 CuCN + 2 CN⁻

3 Cu(CN)₂→ CuCN.Cu(CN)₂ + 3 CN⁻

The above reactions and other related ones are the primary cause of consumption of cyanide in the electroless plating bath. The rate of consumption is related to the concentration of monovalent and divalent copper, the concentration of cyanide ion, the pH of the bath, the reducing agent (formaldehyde) concentration, and the bath temperature. If the concentration of copper ions and reducing agent and the pH of the bath are each maintained at a constant level during the operating life of the bath as is the normal practice commercially, the rate of consumption is dependent only on the concentration of cyanide ion and the temperature of the bath. As set forth above, it has been found that, for a bath having a given composition, there is a direct relation between rate of consumption and the temperature of the bath.

Figure 1 shows a plot of loss of cyanide ion in one hour versus bath temperature for a typical electroless plating bath having the following composition.

| | Parts by Weight |
|---|---|
| cupric chloride | 5.25 |
| formaldehyde | 2.40 |
| EDTA | 20.00 |
| sodium cyanide | 0.0017 |
| sodium hydroxide | 5.00 |
| surfactant | 0.10 |
| water to make | 1000.00 |

The analyses for cyanide content of the bath at the various times and temperatures were carried out using ion specific electrodes and by acidification of aliquots followed by steam distillation of hydrogen cyanide, collection of the distillate in standard alkali solution and back-titration with standard acid to determine the amount of hydrogen cyanide so liberated.

As noted previously, the curve shown in Figure 1 is unique to a bath having the particular composition shown above and is consistently shown by all baths having that particular composition. A similar but different plot will be obtained from a bath having a different composition.

Based on the data shown in Figure 1, a mathematical equation is derived from which loss of cyanide ion at given intervals of time can be calculated for any particular temperature of the bath from which the data shown in the Figure was derived. This mathematical equation is then used as the basis for determining the amount and frequency with which cyanide ion must be added to the bath in order to substantially maintain the cyanide ion concentration at a predetermined level without the need to do any further analysis of aliquots of the bath in order to control the level of cyanide ion.

The addition of the cyanide ion at the requisite intervals of time in accordance with the invention can be carried out manually. However, in a particular and preferred embodiment, the required additions are carried out automatically using a computer controlled system.

Reference is made to Figure 2 which shows in schematic form a control system in accordance with the invention. Electroless copper plating bath (2) is provided with temperature controller (4), temperature sensor probes (6) and (8), and a feed line (10) through which cyanide ion feedstock can be delivered from storage vessel (12) when pump (14) is activated. The temperature of bath (2) is maintained at a predetermined level by a heater control system shown overall as (18). The various components of the computer system (16) are illustrated schematically in Figure 3 as will be discussed further hereinafter. The control of bath temperature is effected as follows. At predetermined intervals signals characteristic of the temperature of the bath (2) are fed by sensor (6) to the heater control wherein a comparator means compares the signals so received to base reference signals characteristic of the predetermined temperature at which it is desired to maintain bath (2). If a difference between the signals received from sensor (6) and the base reference signals is detected by the comparator, the latter generates signals characteristic of the necessary adjustment to be made. These corrective signals are used by the heater control system (18) which activates temperature control means (4) to allow the necessary correction to be made to the bath temperature, either up or down as the case may be. Temperature sensor (8) produces signals characteristic of the bath temperature and these signals are used to monitor the heater control system (18) for proper operation. The above described process of monitoring the temperature of the bath is carried out continuously at very short intervals, generally of about one second, although the frequency of monitoring can vary over a wide range and is not critical to successful operation of the system.

In addition to monitoring the temperature of the bath, the computer system (16) is also programmed to make additions of cyanide ion at predetermined intervals of time based on the mathematical relationship between the loss of cyanide ion versus time for the operating life of the particular bath at the operating temperature which is being employed and monitored as described above. Timer means incorporated in the computer system causes signals to be generated at predetermined periods of time which signals are characteristic of the particular amount of cyanide ion which is to be added at any particular period of time. The signals so generated are fed to sensor means associated with pump (14) to cause said pump to be activated for a length of time sufficient to deliver the predetermined or calculated amount of cyanide ion to bath (2) via feed line (10). Fluid flow sensor means (20) located in the feed line (10) between pump (14) and bath (2) is activated by movement of fluid in the feed line and generates signals which are fed to the computer (16) and serve to confirm that pump (14) is delivering cyanide ion feedstock when activated. The frequency with which the additions of predetermined or calculated amounts of cyanide ion are made can vary over a wide range. Advantageously, the additions are programmed to be made at intervals of the order of 0.01 to 120 minutes and preferably of the order of about 1 minute to about 60 minutes.

Advantageously, the temperature at which the bath (2) is maintained constant in accordance with the invention is in the range of about 25°C. to about 75°C. and, preferably, is within the range of about 30°C. to about 60°C. However, the bath temperature employed in the process of the invention is not critical and the above ranges are given for purposes of illustration only. The optimum temperature in any given instance can be determined by a process of trial and error.

The level of concentration at which the cyanide ion (present typically in the form of the potassium or sodium salt) is maintained is advantageously in the range of about 0.1 to about 100 ppm and, preferably, in the range of about 0.5 to about 50 ppm. However, these concentration ranges are given for purposes of illustration only and are not limiting and the process of the invention can be carried out with concentrations above or below these ranges.

The system of the invention has an additional advantageous feature which centers around the significant and unexpected finding that the rate of loss of cyanide ion is directly proportional to the actual concentration of cyanide ion, i.e. the greater the concentration the greater the rate of consumption. If the amount of cyanide ion added at a given time is greater or less than the amount actually needed at that particular time to maintain the desired level, the error is quickly corrected because of the above factor. Thus, if the amount added is in excess of that required, the increased level of cyanide causes the rate of consumption to increase accordingly and thereby quickly overcome the error. Conversely, if the amount added is less than actually required, the rate of consumption is lower than that at the higher desired level of cyanide ion and the error is again quickly corrected. This self-correcting effect is an added and unexpected advantage in terms of the overall control achieved by the system of the present invention.

Figure 3 shows in schematic form a breakdown of the various components of the computer system shown overall as (16) in Figure 2, the functioning of which system has been discussed above. As shown in Figure 3, microprocessor (22) serves to receive, process and transmit appropriate signals characteristic of a variety of functions. Timer means (24) provides signals to microprocessor (22) at preset intervals which signals are characteristic of the times at which one or other function of the system is to be activated. The RAM/ROM component (26) contains the software for operation of the system. The temperature monitoring component is preferably a cold junction compensated analog/digital converting temperature control system with track and hold features which receives signals from the temperature sensor (8) [see Figure 21, converts these signals from analog to digital mode, transmits the same to microprocessor (22) for calculation of a temperature database used to determine cyanide consumption. These signals are also compared with base reference signals characteristic of the desired temperature level and monitors the proper operation of the heater control system (18).

Computer (22) also generates signals, at predetermined time intervals which are transmitted to pump control component (30), which signals are characteristic of the time component for which pump (14) must be activated to deliver the amount of cyanide ion from storage vessel (12) to bath (2) which amount has been predetermined as required by the bath at the time in question to maintain the desired cyanide level in the bath. The component (30) is provided with the necessary logic to transmit the appropriate signal to the operating mechanism of the pump.

Unit (32) of the system comprises a standard terminal keyboard for accessing the system and video display monitor to permit an operator to set up a program for the overall system, to make any necessary changes to additions thereto and to monitor actual operating parameters of the system during operation thereof. In an alternative embodiment the overall system is entirely preprogrammed and need only respond to alarm conditions such as pump failure, heater failure, empty feedstock reservoir, and the like.

The electronic components necessary to carry out the various functions described above in respect of the systems shown and discussed in regard to Figures 2 and 3 are well known and commercially available. A detailed discussion of the circuits involved in producing the aforesaid functions is accordingly omitted. Illustrative of commercially available components which can be employed in the computer system described above are shown below. It is to be noted that these are given for purposes of exemplification and the invention is not limited to the use of these particular pieces of equipment either individually or in combination.

Illustrative of commercially available timer units is that available under the name DIGI-TIMER from SSAC Inc. Representative of microprocessor units is the mch 18 available from Wintek Corporation and for the ROM/RAM component the mcm 2814p and mcm 6206p units available from Motorola Semiconductors. A typical display unit is that available from Digital Equipment Corporation under the name VT 420 and a typical terminal keyboard is the RS232/RS423 COM-PAC available from Grayhill Inc. Representative of temperature control system components is the unit available from Protec Inc. as model d15d, and representative of pump control system components is the unit available from Crydom Company as a series 6 module.

Programmable computer controlled means for monitoring and adjusting the levels of copper ion, formaldehyde, pH and other parameters of an electroless copper plating bath are already known and commonly used in the art and will not be described in detail herein. Such computer means generally include means for producing base reference signals characteristic of a predetermined level of the parameters to be monitored, sensing means for producing signals characteristic of the actual levels of each parameter in the plating bath, comparator means producing signals responsive to any difference between the signals so produced and the base reference signals, and means sensitive to said comparative response to indicate the need for any necessary adjustment to the actual levels of the various parameters in the bath. Such means may be incorporated into the system of the invention if desired or may be maintained separate therefrom.

The control process of the invention, when employed in the electroless deposition of copper on a substrate such as those employed in the manufacture of printed circuit board, gives rise to a deposited copper layer which has significantly improved properties compared with layers deposited by prior methods. Illustratively, two identical substrates comprising epoxy fiberglass reinforced sheets having copper foil laminated on one side thereof were subjected to electroless copper plating. In the case of both substrates, the coating was carried out using a bath having the following composition:

| | Parts by weight |
|---|---|
| copper sulfate pentahydrate | 9.83 |
| formaldehyde | 1.90 |
| EDTA | 20.00 |
| sodium cyanide | 0.002 |
| sodium hydroxide | 2.80 |
| surfactant | 0.10 |
| additives | 0.02 |
| water to make | 1000.00 |

The bath was maintained at 60°C. In the case of one substrate (A) the deposition was carried out using a computer control system of the invention. A layer of thickness 1.0 mil. was deposited. In the case of the other substrate (B) the deposition to the same thickness was carried out without benefit of a control system of the invention and the cyanide level was maintained in the conventional manner with the cyanide in the caustic soda component which was added to the bath as required. Plating times were of the order of 16 hours in both cases. The following properties were then determined for the copper layer on each substrate after removal of the reinforcing layer by dissolution in concentrated sulfuric acid.

| Property | Substrate | A | B |
|---|---|---|---|
| Tensile strength | | 51,000 psi | 39,000 psi |
| % elongation | | 10 | 7 |

It is to be understood that the above description and exemplification has been given for purposes of illustration only and is not to be considered as limiting. Various modifications which will be readily apparent to one skilled in the art can be made without departing from the scope of the invention which latter is defined only by the claims which follow.

## Claims

1. A process for the electroless deposition of copper onto a substrate surface from an electroless copper depositing bath comprising cupric ions, a reducing agent, a complexing agent and a stabilizing agent comprising cyanide ion, characterised in that the concentration of cyanide ion in the said bath is substantially uniformly maintained at a predetermined level over the course of copper deposition from the bath, by a process which comprises:
(a) establishing, for fixed values of cupric ion concentration, reducing agent concentration and pH of said bath, a characteristic relationship between cyanide ion consumption in the bath and time for a fixed bath temperature;
(b) substantially uniformly maintaining the temperature of the bath at the said fixed temperature;
(c) substantially uniformly maintaining the cupric ion concentration, reducing agent concentration and pH of the bath at the said fixed values thereof; and
(d) adding to the bath over the course of copper deposition therefrom an amount of cyanide ion sufficient to substantially replace the cyanide ion consumed in the bath according to the characteristic relationship established in (a), the addition of the cyanide ion being carried out at time intervals sufficient to maintain substantially uniformly the cyanide ion concentration in the bath at the said predetermined level over the course of copper deposition therefrom.

2. Apparatus for maintaining a predetermined level of cyanide ion stabilizer in an electroless copper plating bath at a constant temperature, which apparatus comprises
an electroless copper plating bath comprising cupric ions, a reducing agent, a complexing agent and a stabilizing agent comprising cyanide ions, the plating bath also comprising heat control means for adjusting the temperature thereof;
storage means containing cyanide ion feedstock and pump means associated with the storage means for delivering cyanide solution via a feed line to the plating bath;
programmable computer means for monitoring the temperature of the plating bath and for controlling the addition of predetermined amounts of cyanide ions at predetermined or calculated intervals, the computer means including
(a) means for producing base reference signals characteristic of a predetermined bath temperature;
(b) sensing means for producing signals characteristic of the temperature of the bath; and
(c) means for producing at predetermined time intervals signals characteristic of predetermined or calculated amounts of cyanide ion feedstock to be added to the bath at the said predetermined time intervals and means sensitive to the signals to activate the pump means to deliver each of the predetermined or calculated amounts at each of the said predetermined intervals.

3. Apparatus according to claim 2, which also comprises flow sensor means located in the feed line between the pump means and the plating tank, the flow sensor means generating signals characteristic of the rate of flow of cyanide ion feedstock in the feed line.

4. Apparatus according to claim 2 or 3, wherein the amount of cyanide ion feedstock added at any given time interval is the amount predetermined or calculated to be necessary at that particular time interval to restore the cyanide ion concentration in the plating bath to the level initially present therein.

5. Apparatus according to claim 2, 3 or 4, which also comprises programmable computer means for monitoring and adjusting the pH and concentrations of cupric ions and formaldehyde in the plating bath, the computer means including means for producing base reference signals characteristic of a predetermined level of each of the aforesaid parameters, sensing means for producing signals characteristic of the actual levels of said parameters in the plating bath, comparator means producing signals responsive to any difference between the signals so produced and the base reference signals and means sensitive to the comparative response to indicate the need for any necessary adjustment to the actual levels of the said parameters in the plating bath.

6. A substrate electrolessly coated with a layer of copper using a process as claimed in claim 1.
